

## 1

2,983,679

## MINERAL OIL CONTAINING A RARE EARTH METAL DIESTER PHOSPHATE

John P. Pellegrini, Jr., and Harold O. Strange, Pittsburgh, Pa., assignors to Gulf Research & Development Company, Pittsburgh, Pa., a corporation of Delaware

No Drawing. Filed Dec. 31, 1958, Ser. No. 784,022

6 Claims. (Cl. 252—32.5)

This invention relates to a new class of chemical compounds which are useful as addition agents to lubricating oils and oil compositions containing the same, and more particularly the invention relates to mineral oil compositions containing a rare earth metal salt of a diester of o-phosphoric acid. By the term "rare earth metal salts," we mean the salts of the elements of atomic numbers 57 to 71, inclusive. The "rare earth" elements thus include lanthanum, cerium, praseodymium, neodymium, samarium, europium, gadolinium, terbium, dysprosium, holmium, erbium, thulium, ytterbium and lutecium. The mineral oil compositions of this invention have improved pour point and viscosity index characteristics.

The viscosity-temperature relationship of a lubricating oil is one of the more important characteristics of an oil in that it is this relationship which is indicative of the relative change in viscosity of an oil at high and low temperatures. As might be expected, the viscosity of a mineral lubricating oil changes rapidly with a change in its temperature. In general, mineral oils tend to become thinner as their temperature increases and thicker as their temperature decreases. The change in viscosity with temperature is greater with some oils than with others. While some change is tolerable, excessive change is undesirable. In motor oils of the type known as crankcase oils, it is desirable for the oil to have a viscosity which is sufficiently high at an elevated temperature to provide adequate lubrication and to prevent excessive oil consumption. On the other hand, the motor oil should have a viscosity which is sufficiently low at atmospheric temperature to provide ease of engine starting. Increasing the high temperature viscosity of an oil while decreasing its low temperature viscosity can be accomplished only by improving the viscosity-temperature relationship, or stated differently, by raising the viscosity index of the oil.

In order to reduce excessive change in viscosity with temperature, various viscosity index improvers have been developed. In the past, for example, polymerized esters of the acrylic series have been used to improve the viscosity-temperature relationship of mineral oils but these esters have not been entirely satisfactory inasmuch as their viscosity index improving characteristics is lost or substantially reduced when the oil in which they are incorporated is subjected to vigorous agitation and high shear rates and stresses. It is believed that the lowering of the viscosity index of an oil containing a long chain polymer as a viscosity index improving agent is a result of such polymer being split into polymers of shorter chain length by the shearing stress, the shorter chain polymers being less effective as viscosity index improvers.

We have found that a rare earth metal salt of a diester of o-phosphoric acid imparts excellent viscosity index improving characteristics to a mineral oil and that the oil thus improved retains its high viscosity index even when subjected to vigorous agitation and high shear rates and stresses. We have found further that a lubricating composition comprising a major amount of a mineral oil

## 2

and a minor amount of a rare earth metal salt of a diester of o-phosphoric acid has a greatly improved pour point.

The lubricating oil to which the viscosity index improving agent is added according to the invention is advantageously a highly refined paraffinic oil. By the term "highly refined paraffinic oil" we mean a petroleum lubricating oil which has been refined by one of the more drastic refining methods known in the art, for example, by conventional aluminum chloride refining or by solvent extraction adapted to remove all or substantially all of the unsaturated and naphthenic constituents of the oil. Aluminum chloride refined or solvent extracted paraffinic base oil, such as a Pennsylvania oil, provides an excellent base oil for the composition of the invention. However, drastically refined Mid-Continent and Gulf Coastal oil may also be used. While the highly refined paraffinic oils are particularly desirable for use in forming crankcase lubricants we do not wish to limit the invention to these oils alone, however, inasmuch as the rare earth metal salt of a diester of o-phosphoric acid as hereinafter defined is also useful in improving the viscosity index and pour point of oils derived from naphthenic and asphaltic crudes.

25 The rare earth metal salts of the o-phosphoric acid esters which can be used in accordance with the invention are those which are soluble in hydrocarbon oils and insoluble in water. In this regard, we prefer to employ a rare earth metal salt of a diester of o-phosphoric acid wherein the ester substituents comprise one short chain 30 aliphatic radical and one long chain aliphatic radical. The short chain radical preferably contains from 1 to 3 carbon atoms and the long chain radical preferably contains from 8 to 20 carbon atoms. The length of the respective chains is determined by the solubility of the resultant compound in mineral oil. The limit of solubility is believed to be reached when the long aliphatic chain contains from 14 to 16 carbon atoms for a saturated group and from 18 to 20 carbon atoms or more for an unsaturated group.

40 The rare earth metal salt of the diester of o-phosphoric acid can be prepared by any suitable method. According to a preferred procedure, the rare earth metal salt of the o-phosphoric acid ester is prepared by reacting a basic rare earth metal compound with an acidic o-phosphoric acid ester. The rare earth metal compound is employed in an amount sufficient to effect complete neutralization of the o-phosphoric acid ester. In some instances, the neutralization reaction takes place spontaneously, or substantially so, with the evolution of heat. In other instances, however, it is required to add additional heat to effect complete neutralization. In effecting complete neutralization, it is preferred to maintain the reaction temperature below about 220° F. in order to avoid appreciable decomposition of the resulting salt. After salt 45 formation is substantially complete, the mixture is further heated for a time sufficient to expel the water of neutralization. The use of a slight vacuum at this point facilitates dehydration. Thereafter, the dehydrated product is filtered to separate out any unreacted rare earth metal compound. In some instances, it is desirable to prepare an alkali metal salt of the organic phosphate and thereafter prepare the rare earth metal salt by metathesis of the alkali metal salt with a water-soluble salt of the rare earth metal such as the nitrate, chloride or sulfate, as appropriate.

50 The rare earth metal compound used in preparing the corresponding metal salt of the diester of o-phosphoric acid can be either a relatively pure compound or it can be a mixture of the rare earth compounds such as are found in monazite and bastnasite. The following table shows the composition of rare earths in typical commercial rare earth salts.

3  
TABLE I

|                                  | Composition of Rare Earths, Wt. Percent as Oxides |                                |                                 |                                |                                |        |
|----------------------------------|---------------------------------------------------|--------------------------------|---------------------------------|--------------------------------|--------------------------------|--------|
|                                  | Ce <sub>2</sub> O <sub>3</sub>                    | La <sub>2</sub> O <sub>3</sub> | Pr <sub>6</sub> O <sub>11</sub> | Nd <sub>2</sub> O <sub>3</sub> | Sm <sub>2</sub> O <sub>3</sub> | Others |
| Rare earth salts from monazite   | 48                                                | 24                             | 6                               | 19                             | 2                              | 1      |
| Rare earth salts from bastnasite | 48                                                | 37                             | 3.5                             | 10                             | 1                              | 0.6    |

While the individual rare earth metal oxides can successfully be employed in preparing the salt of the diester of o-phosphoric acid, compounds of the individual elements are more expensive because of the increasing difficulty of separating the individual elements. Therefore, from an economic standpoint it is desirable to prepare the rare earth metal salt of a diester of o-phosphoric acid by neutralizing the o-phosphoric acid ester with a mixture of the rare earth oxides.

The acidic o-phosphoric esters used in making the rare earth metal salts for the purposes of the invention also may be prepared in any suitable manner. For example, a mixture of a higher monohydric alcohol containing from 8 to 20 carbon atoms, a monohydric alcohol containing from 1 to 3 carbon atoms and phosphorus pentoxide may be refluxed for several hours. The complex mixture of mono, di and tri esters may be distilled to obtain individual pure compounds.

According to another embodiment, phosphorus oxychloride is reacted with a monohydric alcohol containing from 1 to 3 carbon atoms to form the corresponding phosphoryl dichloride which is thereafter reacted with a monohydric alcohol containing from 8 to 20 carbon atoms to form a phosphoryl monochloride which is subsequently hydrolyzed to form the desired phosphoric acid diester containing a C<sub>1</sub> to C<sub>3</sub> aliphatic radical and a C<sub>8</sub> to C<sub>20</sub> aliphatic radical. Examples of the short chain alcohols are methyl alcohol, ethyl alcohol, n-propyl alcohol, isopropyl alcohol and allyl alcohol. Examples of the long chain alcohols are n-octyl, iso-octyl, nonyl, decyl, n-dodecyl (lauryl), tetradecyl, n-hexadecyl, n-octadecyl (stearyl), n-octadecenyl (oleyl), n-octadecadienyl (linoleyl) and eicosyl alcohols. The alcohols need not be pure as mixtures of two or more can be used.

Organic phosphates that form suitable rare earth metal salts for the purposes of this invention are diesters of o-phosphoric acids whose two ester substituents are aliphatic radicals one of which contains from 1 to 3 carbon atoms and the other contains from 8 to 20 carbon atoms. Examples of such organic diesters of phosphoric acids are methyl n-octyl, ethyl n-octyl, n-propyl n-octyl, isopropyl iso-octyl, allyl iso-octyl, methyl nonyl, ethyl nonyl, propyl nonyl, methyl decyl, ethyl decyl, propyl decyl, methyl dodecyl, ethyl n-dodecyl (ethyl lauryl), allyl n-dodecyl, ethyl tetradecyl, ethyl n-hexadecyl, ethyl n-octadecyl (ethyl stearyl), allyl n-octadecyl, ethyl n-octadecenyl (ethyl oleyl) ethyl n-octadecadienyl (ethyl linoleyl), and ethyl eicosyl esters of o-phosphoric acid.

Specific examples of especially effective agents for the purposes of the invention are the oil-soluble lanthanum and neodymium salts of ethyl oleyl acid orthophosphates. Other salts included by the invention are the lanthanum, neodymium, praseodymium, cerium and samarium salts of ethyl n-octyl, ethyl iso-octyl, ethyl decyl, ethyl n-dodecyl (lauryl), ethyl n-octadecyl (stearyl) and ethyl n-octadecenyl acid orthophosphates.

The preparation of the salts for use in the compositions of the invention are illustrated by the following specific examples.

#### EXAMPLE I

##### *Lanthanum ethyl oleyl orthophosphate*

Into a 3 liter round bottom flask equipped with a mechanical stirrer, condenser and dropping funnel are placed 89.2 gm. of ethyl oleyl acid orthophosphate, 400

ml. of water and 250 ml. of 95% ethanol. To the mixture thus formed are added, with stirring, 9.49 gm. sodium hydroxide in 200 ml. of water. The temperature of the reaction is maintained at about 25° C. To the reaction mass thus formed are slowly added 34.2 gm. of lanthanum nitrate hexahydrate in 200 ml. of water with rapid stirring, the temperature of the metathesis reaction being maintained at about 25° C. A gummy yellow precipitate is formed. The water is decanted from the reaction mass and thereafter the precipitate is dissolved in hexane, solution being facilitated by the application of a small amount of heat. Thereafter, the product is filtered to remove any undissolved solids. Solvent is then stripped from the filtrate. When the solvent is completely removed, an opaque yellowish rubber-like product comprising lanthanum ethyl oleyl phosphate is obtained. Analysis of the product shows it to compare favorably with the theoretical analysis of lanthanum ethyl oleyl orthophosphate as follows:

|            | Found | Theoretical |
|------------|-------|-------------|
| Carbon     | 50.83 | 56.95       |
| Hydrogen   | 10.31 | 9.49        |
| Phosphorus | 5.75  | 7.35        |
| Lanthanum  | 10.07 | 11.00       |

The rare earth metal salts of the o-phosphoric acid esters can be employed per se or they can be added to the lubricating oil in the form of a mineral oil concentrate. In preparing the mineral oil concentrate, the rare earth metal salt can be prepared in an organic solvent which can be flashed from the oil after formation of the concentrate. Organic solvents suitable for this purpose include hexane, isooctane, naphtha, benzene, toluene, carbon tetrachloride, and the like. When a mineral oil concentrate is prepared first, the concentrate can be added directly to the oil to be improved or it can be admixed with one or more other improving agents. Regardless of whether the rare earth metal salt of the o-phosphoric acid ester is employed per se or in the form of a mineral oil concentrate, an amount is used sufficient to impart viscosity index and pour point improving characteristics to the oil. For example, the rare earth metal salts are useful when employed in amounts of about 0.1 to about 5 percent by weight. Amounts in excess of 5 percent are generally undesirable because the oil becomes too viscous for satisfactory use as crankcase lubricant. Excellent results have been obtained by the use in petroleum distillates such as, SAE 10 and SAE 20 lubricating oil, of amounts of the salts between 0.1 and 0.5 percent by weight of the composition. It will be understood that the optimum amount will vary according to the particular mineral oil and according to the conditions to which the oil is subjected.

The following examples illustrate the preparation of mineral oil concentrates of the various rare earth metal salts of o-phosphoric acid esters. The mineral oil used in the examples is an SAE 10 highly refined paraffinic oil having a viscosity of 171 and 45.2 SUS at 100° F. and 210° F., respectively; a viscosity index of 110; a flash point of 465° F.; a fire point of 505° F.; a pour point of +10° F.; and a color, ASTM Union of 2 minus.

#### EXAMPLE II

##### *Neodymium ethyl oleyl orthophosphate*

Into a 2 liter round bottom flask equipped with a mechanical stirrer and reflux condenser are placed 970 gm. of an SAE 10 highly refined paraffinic oil. To the mass of oil are added 4.00 gm. of neodymium oxide and 26.65 gm. of ethyl oleyl o-phosphoric acid with rapid stirring. The addition of several cubic centimeters of water at this point is advantageous in order to increase the speed of the reaction. The reaction mass thus formed is heated at 75° C. for several hours with continued

stirring. Heating is continued for from 1 to 3 or 4 hours or until the reaction is substantially complete. When the reaction is complete, the water is removed from the reaction product under a reduced pressure at about 75° to 80° C. The heated solution is then filtered to remove any unreacted neodymium oxide. The filtered oil thus obtained is light in color and is fairly viscous, comprising a 3% solution of neodymium ethyl oleyl orthophosphate in mineral oil.

### EXAMPLE III

#### *Lanthanum ethyl oleyl orthophosphate*

Into a 3 liter round bottom flask are placed 970 gm. of an SAE 10 highly refined paraffinic oil, 26.7 gm. of ethyl oleyl o-phosphoric acid and 4.0 gm. of lanthanum oxide. To this mixture are added 5 ml. of water followed by heating at 80° C. with stirring for 3 hours. The water is then removed by heating under a vacuum at 80° C. The heated product is then filtered to remove excess lanthanum oxide. When the oil cools it becomes quite viscous but is still sufficiently fluid to flow. The product comprises a 3% solution of lanthanum ethyl oleyl orthophosphate in mineral oil.

### EXAMPLE IV

#### *Lanthanum ethyl lauryl orthophosphate*

Into a 2 liter round bottom flask are placed 760 gm. of an SAE 10 highly refined paraffinic mineral oil, 34.6 gm. of ethyl lauryl phosphate and 10 gm. of lanthanum oxide. To this mixture are added 10 ml. of water followed by heating for 4 hours at 95° C. Upon completion of the reaction, the water is removed by heating under a vacuum at about 95° C. The heated product is then filtered to remove excess lanthanum oxide. The filtered oil product which becomes quite viscous when it cools comprises a 5% solution of lanthanum ethyl lauryl orthophosphate in mineral oil.

### EXAMPLE V

#### *Cerium ethyl oleyl orthophosphate*

Into a 2 liter flask are placed 1170 gm. of an SAE 10 highly refined paraffinic mineral oil, 26.7 gm. of ethyl oleyl orthophosphate, 30 ml. of water and cerium hydroxide obtained by reacting 17 gm. of cerium nitrate with ammonium hydroxide. The reaction mass is heated to 75° to 80° C. and dehydrated as in the previous examples. The product comprises a 2.5% solution of cerium ethyl oleyl orthophosphate in mineral oil.

### EXAMPLE VI

#### *Praseodymium methyl oleyl orthophosphate*

Praseodymium oxide and methyl oleyl orthophosphate are admixed with a small amount of water and added to an SAE 10 highly refined paraffinic mineral oil as in Example IV. Upon heating and removal of the water as in Example IV, an oil solution of praseodymium methyl oleyl orthophosphate is obtained.

### EXAMPLE VII

#### *Samarium ethyl oleyl orthophosphate*

The procedure of Example III is followed except

samarium oxide is substituted for lanthanum oxide. The product comprises an oil solution of samarium ethyl oleyl orthophosphate.

### EXAMPLE VIII

#### *Lanthanum ethyl isoctyl orthophosphate*

The procedure of Example IV is followed except ethyl isoctyl orthophosphate is substituted for ethyl lauryl phosphate. The product comprises an oil solution of lanthanum ethyl isoctyl orthophosphate.

### EXAMPLE IX

#### *Neodymium methyl eicosyl orthophosphate*

The procedure of Example II is followed except methyl eicosyl o-phosphoric acid is substituted for the ethyl oleyl o-phosphoric acid. The resulting product comprises an oil solution of neodymium methyl eicosyl orthophosphate.

### EXAMPLE X

#### *Lanthanum propyl oleyl orthophosphate*

The procedure of Example IV is followed except propyl oleyl orthophosphate is substituted for ethyl lauryl phosphate. The resulting product comprises an oil solution of lanthanum propyl oleyl orthophosphate.

It will be understood that the foregoing examples are illustrative only and that other rare earth metal salts of diester orthophosphates wherein the ester substituents comprise one short chain aliphatic radical containing from 1 to 3 carbon atoms and one long chain aliphatic radical containing from 8 to 20 carbon atoms can be employed. Specific examples of such other salts include the europium, gadolinium, terbium, dysprosium, holium, erbium, thulium, ytterbium and lutecium salts of methyl oleyl, ethyl oleyl, propyl oleyl, ethyl isoctyl, ethyl eicosyl and allyl lauryl orthophosphoric acid.

While the preparation of the rare earth metal salts according to the procedure given in Examples II to X utilizes a mineral oil solvent, it will be understood that the rare earth metal salts useful for the purposes of the invention can be obtained in the free state, as in Example I, just as readily as they are obtained in mineral oil blends. To obtain the free rare earth metal salt of a diester orthophosphate, a more volatile solvent, such as hexane, benzene and carbon tetrachloride, is used in place of a mineral oil and is flashed off either before or after the formation of the rare earth salt.

To demonstrate the effectiveness of the rare earth metal salts of the type described above in the mineral oil compositions contemplated by this invention, we have conducted several comparative tests, the results of which are listed below, with representative mineral oils alone and with the same oils blended with various representative rare earth metal salts of diester orthophosphates. These tests were conducted with highly refined paraffinic mineral oils of SAE 10 and SAE 25 grade. The improvement produced by the improving agents of the present invention in the viscosity index of mineral oils to which they are added is clearly shown by the illustrative data in Table II.

TABLE II

| Composition, Percent by Weight    | A     | B     | C     | D     | E     | F     | G     | H     | I     | J     | K     |
|-----------------------------------|-------|-------|-------|-------|-------|-------|-------|-------|-------|-------|-------|
| SAE 10 Mineral Oil                | 100   |       | 99.9  | 99.75 | 99.75 |       | 99.9  | 99.85 | 99.8  | 99.75 | 99.5  |
| SAE 25 Mineral Oil                |       | 100   |       |       |       |       |       |       |       |       | 99.5  |
| Neodymium ethyl oleyl o-phosphate |       |       | 0.1   | 0.25  |       | 0.1   | 0.15  | 0.2   | 0.25  | 0.5   |       |
| Lanthanum ethyl oleyl o-phosphate |       |       |       |       | 0.25  |       |       |       |       |       | 0.5   |
| VISCOSITY DATA                    |       |       |       |       |       |       |       |       |       |       |       |
| Viscosity, cs.                    |       |       |       |       |       |       |       |       |       |       |       |
| at 100° F                         | 36.55 | 77.76 | 43.80 | 64.13 | 38.85 | 83.85 | 94.37 | 104.8 | 123.6 | 234.1 | 83.70 |
| at 210° F                         | 5.80  | 7.28  | 12.60 | 12.60 | 10.64 | 12.18 | 14.01 | 16.67 | 30.85 | 18.43 |       |
| Viscosity Index                   | 110   | 108   | 131   | 152   | 173   | 117   | 123   | 129   | 132   | 133   | 154   |

The data in the above Table II clearly shows that even as little as 0.25 percent of the neodymium and lanthanum salts of ethyl oleyl o-phosphate greatly improves the viscosity index of the mineral oil.

The improvement in pour point is shown by the data in Table III.

TABLE III

| SAE 10 Mineral Oil                                           | ASTM Pour Point, °F. |
|--------------------------------------------------------------|----------------------|
| SAE 10 Mineral Oil + 0.25% neodymium ethyl oleyl o-phosphate | +10                  |
| SAE 10 Mineral Oil + 0.25% lanthanum ethyl oleyl o-phosphate | -20                  |
|                                                              | +5 15                |

While the neodymium salt is more effective than the lanthanum salt, the improvement with such a small amount of additive is nevertheless striking.

The ability of the oil compositions of the invention to retain their improved viscosity index characteristics even though subjected to prolonged ultrasonic irradiation is demonstrated by the data shown in Table IV. These tests were conducted with a highly refined paraffinic mineral oil of SAE 25 grade. Several comparative tests were made with (1) the mineral oil alone, (2) with the same oil blended with a representative rare earth metal salt of a diester orthophosphate and (3) with the mineral oil containing a commercially available viscosity index improving agent of the polymerized acrylic series.

TABLE IV

| Composition, Percent by Weight    | L                           | M    | N    | O    |
|-----------------------------------|-----------------------------|------|------|------|
| SAE 25 Mineral Oil                | 100                         | 99.9 | 99.5 | 95.0 |
| Neodymium ethyl oleyl o-phosphate |                             | 0.1  | 0.5  |      |
| Polymerized acrylic ester         |                             |      |      | 5.0  |
| Viscosity Data:                   |                             |      |      |      |
| Irradiation time (minutes):       | Viscosity, c.s., and VI at— |      |      |      |
|                                   | ° F.                        |      |      |      |
| 0                                 | 100 78.81 100.2 263.0 95.54 |      |      |      |
|                                   | 210 9.51 11.97 34.29 14.34  |      |      |      |
|                                   | VI 106 115 136 136          |      |      |      |
| 30                                | 100 78.68 97.14 207.3 77.07 |      |      |      |
|                                   | 210 9.50 11.82 33.00 10.09  |      |      |      |
|                                   | VI 106 116 138 118          |      |      |      |
| 60                                | 100 79.21 95.71 218.6 75.07 |      |      |      |
|                                   | 210 9.47 11.45 32.85 9.81   |      |      |      |
|                                   | VI 105 113 137 117          |      |      |      |
| 90                                | 100 78.19 95.00 193.0 75.61 |      |      |      |
|                                   | 210 9.49 11.56 31.50 9.92   |      |      |      |
|                                   | VI 107 116 139 117          |      |      |      |
| 120                               | 100 78.41 95.25 169.1 74.10 |      |      |      |
|                                   | 210 9.50 11.71 25.58 9.65   |      |      |      |
|                                   | VI 107 118 139 116          |      |      |      |

The improvement obtained in viscosity index by the improving agents of the present invention is clearly shown by the illustrative data in Table IV. It will be noted that even after 120 minutes of ultrasonic irradiation, the compositions of the invention, i.e., Compositions M and N, retained their improved viscosity indices. Contrariwise, the SAE 25 oil which contained the commercially available polymerized acrylic ester did not retain its initial viscosity index even though the agent was present in amounts 10 to 50 times greater than the improving agent of the invention. It will be noted further that while ultrasonic irradiation caused some decrease in the viscosity of the compositions of the invention both at 100° F. and at 210° F., the irradiated compositions in every instance had viscosities considerably above the viscosity of the base oil. On the other hand, the base oil con-

taining the polymerized acrylic ester after ultrasonic irradiation had a viscosity even less than the viscosity of the base oil when measured at 100° F. and substantially the same viscosity when measured at 210° F. The data thus obtained in the ultrasonic shear stability tests indicate that the rare earth metal salts of diester o-phosphates are surprisingly stable even when subjected to vigorous agitation and high shear rates and stresses.

An inspection of the physical properties of an SAE 10 mineral lubricating oil and the same lubricating oil containing 0.25 percent by weight of neodymium ethyl oleyl o-phosphate and 0.25 percent by weight of lanthanum ethyl oleyl o-phosphate are as follows:

|                          | Lubricating Oil | Lubricating Oil + 0.25% neodymium ethyl oleyl o-phosphate | Lubricating Oil + 0.25% lanthanum ethyl oleyl o-phosphate |
|--------------------------|-----------------|-----------------------------------------------------------|-----------------------------------------------------------|
| Viscosity, SUS:          |                 |                                                           |                                                           |
| at 100° F.               | 171             | 207                                                       | 181                                                       |
| at 210° F.               | 45.2            | 68.8                                                      | 68.9                                                      |
| Viscosity Index:         |                 |                                                           |                                                           |
| Flash Point, OC: ° F.    | 110             | 152                                                       | 173                                                       |
| Fire Point OC: ° F.      | 465             | 450                                                       | 445                                                       |
| Pour Point, ° F.         | 505             | 505                                                       | 495                                                       |
| Color, ASTM Union        | +10             | -20                                                       | +5                                                        |
| Neutralization Value:    | 2 minus         | 2 minus                                                   | 2 minus                                                   |
| ASTM D-974               | ≤ 0.01          | 0.17                                                      | 0.11                                                      |
| Ash, ASTM D-432, percent | ≤ 0.01          | 0.05                                                      | 0.06                                                      |

The lubricating oil composition of this invention can contain other addition agents normally added to lubricating oils for a specific purpose such as an oiliness and extreme pressure agent, an anti-oxidant, a corrosion inhibitor, a foam suppressant, a dye, a sludge inhibitor, and the like.

While our invention has been described with reference to various specific examples and embodiments it will be understood that the invention is not limited to such examples and embodiments and may be variously practiced within the scope of the claims hereinafter made.

We claim:

1. A lubricating composition comprising a major amount of a mineral oil and a minor amount, sufficient to impart improved viscosity index characteristics to the composition, of a rare earth metal salt of a diester of o-phosphoric acid wherein the rare earth metal is an element having an atomic number from 57 to 71 and the ester substituents comprise one aliphatic radical containing from 1 to 3 carbon atoms and one aliphatic radical containing from 8 to 20 carbon atoms.

2. The composition of claim 1 wherein said minor amount is about 0.1 to 5 percent by weight of the composition.

3. A lubricating composition comprising a major amount of a mineral lubricating oil and a minor amount, sufficient to impart improved viscosity index characteristics to the composition, of a lanthanum salt of a diester of o-phosphoric acid wherein the ester substituents comprise one aliphatic radical containing from 1 to 3 carbon atoms and one aliphatic radical containing from 8 to 20 carbon atoms.

4. A lubricating composition comprising a major amount of a mineral lubricating oil and a minor amount, sufficient to impart improved viscosity index characteristics to the composition, of a neodymium salt of a diester of o-phosphoric acid wherein the ester substituents comprise one aliphatic radical containing from 1 to 3 carbon atoms and one aliphatic radical containing from 8 to 20 carbon atoms.

5. A lubricating composition comprising a major

amount of a mineral lubricating oil and a minor amount, sufficient to impart improved viscosity index characteristics to the composition, of lanthanum ethyl oleyl orthophosphate.

6. A lubricating composition comprising a major amount of a mineral lubricating oil and a minor amount, sufficient to impart improved viscosity index characteristics to the composition, of neodymium ethyl oleyl orthophosphate.

## References Cited in the file of this patent

## UNITED STATES PATENTS

|           |                   |               |
|-----------|-------------------|---------------|
| 2,228,658 | Farrington et al. | Jan. 14, 1941 |
| 2,285,853 | Downing et al.    | June 9, 1942  |
| 2,480,673 | Reiff et al.      | Aug. 30, 1949 |

## OTHER REFERENCES

Chem. Abstracts, vol. 52, 18064 g, Nov. 10, 1958.